

# UNITED STATES PATENT OFFICE.

ALBERT PRUESSMAN, OF BERWYN, ILLINOIS, ASSIGNOR TO WESTERN ELECTRIC COMPANY, INCORPORATED, OF NEW YORK, N. Y., A CORPORATION OF NEW YORK.

## CONDENSER AND METHOD OF MAKING THE SAME

1,275,468.

Specification of Letters Patent. Patented Aug. 13, 1918.

No Drawing.

Application filed July 27, 1917. Serial No. 183,181.

To all whom it may concern:

Be it known that I, ALBERT PRUESSMAN, a citizen of the United States, residing at Berwyn, in the county of Cook and State of Illinois, have invented certain new and useful Improvements in Condensers and Methods of Making the Same, of which the following is a full, clear, concise, and exact description.

10 This invention relates to condensers and a method of making the same, its object being to provide an improved method of treating condensers to prevent a permanent change in their electrical constants as a result of 15 normal temperature changes.

In composite circuits, which are used for the simultaneous sending of telephone and telegraph messages, the requirements are such as to demand condensers which are 20 very closely balanced in electrical constants with respect to each other. Also in connection with various other electrical circuits or networks, there is a considerable demand for condensers, the electrical constants of which 25 are necessarily held to very close limits in order that the circuits may function properly. By following a process of selection, it is possible to obtain groups of condensers which initially meet the various requirements, but experience has shown that such 30 condensers, even though made in the same manner and in fact in the same lot, may vary considerably from each other after being subjected to temperature changes to be expected under normal operating conditions. It is, therefore, the object of the 35 present invention to provide a method of treatment which, when applied to the standard type of condensers, will insure that their electrical constants are not permanently affected to an appreciable amount by normal changes in temperature.

The type of condensers most commonly used in telephone practice consists of alternate 45 strips or layers of metal foil and insulating material, such as paper, rolled into a cylindrical or elliptical form. After this unit is wound, it is given a treatment to make it impervious to moisture. Various methods 50 are employed to attain this result, one which has been found to be particularly satisfactory being described in detail in United States Patent 1,127,513, granted to the applicant on February 9, 1915. This method

consists essentially in baking the wound unit 55 to expel all moisture, and then boiling it in melted paraffin wax or an equivalent material. As the unit is allowed to cool, it is shaped by slight pressure applied to the flat sides thereof, after which it is dipped 60 into an insulating compound and then placed in a metal container, which is later completely filled with the insulating compound.

The additional treatment contemplated 65 by this invention consists in placing the treated unit in an oven, which is maintained at a temperature greater than the melting point of the impregnating wax and leaving it at this temperature for a given period of 70 time, after which it is allowed to cool. During this treatment, any stresses, due to unequal winding or unequal pressures during the shaping process, become equalized and the unit is free to take its natural shape, or, 75 so to speak, to take a permanent set, after which there will be no further tendency for change in shape, even though the impregnating wax is in a fluid state. In the case of condensers which are impregnated with 80 a paraffin wax, the solidifying temperature of which is approximately 120° F., a satisfactory treatment has been found to consist in placing the condensers in an upright position in an oven, the temperature of which 85 is maintained at approximately 140° F., and leaving them there for a period of from four to six hours, after which they are allowed to cool. Extensive tests made on condensers so treated indicate that no appreciable 90 change of a permanent nature will take place as a result of temperature changes such as would be experienced under normal operating conditions.

What is claimed is:

1. The method of treating a condenser comprising an impregnated unit, which consists in heating said impregnated unit to a temperature greater than the melting point of the impregnating compound, and maintaining the unit at such temperature for a period of time sufficient to allow the unit to assume its natural shape.

2. The method of treating a condenser comprising a unit impregnated with a paraffin compound, which consists in heating the impregnated unit to a temperature of not less than 120° F., and maintaining said unit at

this temperature for a period of not less than three hours.

3. The method of treating a condenser comprising a unit impregnated with a paraffin compound, which consists in placing the impregnated unit in an upright position in an oven heated to a temperature

of 140° F., and maintaining it at this temperature for a period of substantially four hours.

In witness whereof I hereunto subscribe my name this 25th day of July, A. D. 1917.

ALBERT PRUESSMAN.

DISCLAIMER.

1,275,468.—*Albert Pruessman, Berwyn, Ill. CONDENSER AND METHOD OF MAKING THE SAME.* Patent dated August 13, 1918. Disclaimer filed June 15, 1920, by the patentee, the assignee, *Western Electric Company, Incorporated*, consenting.

Enters this disclaimer—

“To claims 1, 2, and 3 of said Letters Patent, which are in the following words; to wit:

“1. The method of treating a condenser comprising an impregnated unit, which consists in heating said impregnated unit to a temperature greater than the melting point of the impregnating compound, and maintaining the unit at such temperature for a period of time sufficient to allow the unit to assume its natural shape.

“2. The method of treating a condenser comprising a unit impregnated with a paraffin compound, which consists in heating the impregnated unit to a temperature of not less than 120° F., and maintaining said unit at this temperature for a period of not less than three hours.

“3. The method of treating a condenser comprising a unit impregnated with a paraffin compound, which consists in placing the impregnated unit in an upright position in an oven heated to a temperature of 140° F., and maintaining it at this temperature for a period of substantially four hours.”

[Official Gazette July 13, 1920.]